

## UNITED STATES PATENT OFFICE

1,954,000

## ANODIC COATING OF ZINC BASE METALS

Edward Cushman Truesdale and Ernest John Wilhelm, Palmerton, Pa., assignors to The New Jersey Zinc Company, New York, N. Y., a corporation of New Jersey

No Drawing. Application November 14, 1932,  
Serial No. 642,611

20 Claims. (Cl. 204—1)

This invention relates to the coating of zinc base metals by anodic action, and has for its object the provision of an improved method of producing useful anodic coatings on such metals, 5 as well as the provision, as new articles of commerce, of zinc base metals so coated. By "zinc base metal" we mean metals and alloys composed principally of zinc.

The invention is particularly concerned with 10 the production of anodic coatings on zinc and zinc base alloys for the purpose of protection, ornamentation, or of serving as a base for the application of paints, lacquers and the like so as to secure good adhesion of the latter. Ordinary 15 commercial zinc (in particular, rolled or strip zinc), zinc base alloys such as die-casting alloys containing over 90% zinc (for example, the alloys of United States Patents Nos. 1,596,761, 1,663,215, 1,779,525, 1,852,434, 1,852,441 and 1,852,442), and 20 wrought zinc base alloys (for example, the alloys of United States Patents Nos. 1,716,599, 1,832,653, 1,832,733 and 1,835,450) may be advantageously 25 coated by the method of the invention. Numerous other zinc base alloys, particularly those containing small amounts of copper and/or aluminum, are likewise amenable to treatment in accordance 30 with the invention.

In our copending application for Letters Patent of the United States, Serial No. 642,608, filed 35 November 14, 1932, we have disclosed the production of anodic coatings on zinc from strongly basic electrolytes, such as 0.2N to 1.0N sodium hydroxide solutions (pH value of about 13.3 or more). In the course of our investigations, we 40 have discovered that alkaline electrolytes of a slightly lower hydroxyl ion concentration and containing a compound of an amphoteric metal yield anodic coatings on zinc that are characteristically different from those yielded by the 45 strongly alkaline electrolytes of our aforementioned application. Alkaline solutions of the oxides or hydroxides of zinc, aluminum, beryllium and tin (or aqueous solutions of alkali zincates, aluminates, beryllates and stannates) are examples of such alkaline electrolytes containing 50 amphoteric metal compounds. When the concentration of free alkali exceeds a certain amount, in most cases about 0.1N (pH about 13), these amphoteric metal electrolytes behave essentially 55 like simple solutions of an alkali hydroxide (e. g. sodium hydroxide) of the same pH value, and yield dark coatings composed essentially of zinc oxide. If, however, the hydroxyl ion concentration of such alkaline solutions of these amphoteric metals be lowered appreciably below a pH

value of 13 (the exact change of pH depending upon the concentration of amphotolyte), the anodic coatings obtained on zinc are lighter in color, and may contain, in appropriate cases, small amounts of basic compounds of metals other than 30 zinc (e. g. alumina from a sodium aluminate solution). In the case of the true amphotolytes, if the hydroxyl ion concentration is still further reduced, say into the region of pH values of 10 to 12, the anodic coatings obtained from alkaline 35 solutions of these amphotolytes become loose, white and flocculent and consist mainly of the amphoteric metal hydroxide. Such anodic deposits are poorly adherent, and are of little, if any, practical 40 value.

Based on the foregoing discoveries, the method of the present invention involves subjecting a zinc base metal, as anode, to electrolytic treatment in an alkaline electrolyte containing a compound of an amphoteric metal and having a hydroxyl ion concentration sufficient to yield a dense and adherent coating on the zinc anode while insufficient to completely dominate the anion of the amphotolyte. Throughout this specification and the appended claims, we include in 50 the class of amphoteric metals not only the true amphotolytes, that is to say, those metals that form oxides capable of acting as acids or bases without change of valence (e. g. tin, aluminum, beryllium etc.), but also those metals forming oxides 55 which are soluble in both acids and bases, the metal, however, showing different valences in the two solvents (e. g. chromium, tungsten etc.); which metals may be described as pseudo-amphotolytes. The amphoteric metal electrolyte of 60 the invention may be an aqueous solution of the salt formed by the combination of a strong base (such as the hydroxide of an alkali or alkaline-earth metal) with the hydroxide or oxide of an amphoteric metal (which reacts as a weak acid 65 in such a combination). On account of hydrolysis, such a solution in the case of the true amphotolytes has a relatively high hydroxyl ion concentration approximating a pH value of 13. In accordance with the principle of the present 70 invention the hydroxyl ion concentration of the true amphoteric metal electrolytes is preferably maintained at a pH value of about 12 to about 13, although under certain conditions of operation and with certain pseudo-amphotolytes, the pH value may be below 12 and may approximate neutrality. The concentration of the amphoteric metal compound present in the electrolyte will 75 be determined, to some extent, by the critical limit 80

its of hydroxyl ion concentration hereinbefore mentioned.

Since the anodic coating of the invention usually reproduces, in minute detail, the surface markings originally present on the zinc article, the appearance of the coating may be improved by buffing the zinc article before anodic treatment. This buffing procedure may advantageously be of the same character as used on zinc prior to electroplating. Other preliminary treatment, such as sand-blasting or etching which, like buffing, removes a surface film especially likely to be present on cast zinc surfaces, may be employed to facilitate the subsequent anodic treatment. Such preliminary surface treatment of the zinc article, may, of course, be dispensed with if desired.

The zinc article should be appropriately cleaned prior to anodic treatment. This cleaning may be advantageously accomplished in a trisodium phosphate solution containing about six ounces per gallon of water (45 grams per liter of water). This solution is used hot as an electro-cleaner, with the zinc article to be cleaned as the cathode, and with sufficient current to produce copious gassing. When used in this manner, grease (e. g. acquired during rolling or buffing) and loose dirt are completely removed after one-half to three minutes of cleaning. After cleaning, the zinc article is rinsed in hot and then in cold water to remove the residual cleaning solution; following which the zinc article is ready for anodic treatment.

Cathodes of nickel, iron or other metal or alloy insoluble in the alkaline amphoteric metal electrolyte may be used in practicing the invention. The electrolytic treatment is carried out at room temperature and is started at about 6 volts, which may be raised to 30 volts or higher in case the current density decreases due to polarization. The duration of treatment is dependent to some extent upon the composition of the electrolyte, but is usually from 3 to 10 minutes. The anodic coating produced is firm, dense and adherent and varies in color depending upon the amphotolyte used.

The following table gives the composition of several alkaline solutions of amphoteric metal hydroxides, and descriptions of the anodic coatings obtained therefrom by the practice of the invention:

| Solution       | Conc. free NaOH      | Conc. amphotolyte gms. per liter                                                                                 | Color of coating |
|----------------|----------------------|------------------------------------------------------------------------------------------------------------------|------------------|
| Aluminate..... | 2.2 grams per liter. | 3.5 Al <sub>2</sub> O <sub>3</sub> .....                                                                         | White.           |
| Do.....        | 4.4 grams per liter. | 7.1 Al <sub>2</sub> O <sub>3</sub> .....                                                                         | Gray-white.      |
| Stannate.....  | pH 12.8.....         | 50 Na <sub>2</sub> SnO <sub>3</sub> .....<br>3H <sub>2</sub> O.....<br>600 K <sub>2</sub> CrO <sub>4</sub> ..... | Gray.            |
| Chromate.....  |                      |                                                                                                                  | Greenish-yellow. |

The anodic coatings of the invention not only protect the zinc or zinc alloy from corrosion but are also useful for decoration. These coatings may also be used as a base to increase the adherence of paint, enamel, lacquer etc. The light-colored anodic coatings produced in accordance with the invention may be given various colors by dyeing. The dyeing may take place during the electrolytic treatment by solution of the dye in the electrolyte or dyeing may be carried out by immersion of the coated article in an appropriate solution of the dye.

We claim:

1. As a new article of commerce, a zinc base metal having a thin, dense and firmly adherent anodic coating containing a compound of an amphoteric metal other than zinc.

2. As a new article of commerce, a zinc base metal having a thin, dense and firmly adherent anodic coating containing a compound of zinc and a compound of another amphoteric metal. 30

3. As a new article of commerce, a zinc base metal having a thin, light-colored and firmly adherent anodic coating containing compounds of zinc and another amphoteric metal. 85

4. The method of producing a coating on a zinc-base metal which comprises subjecting the metal as anode to electrolytic treatment in an alkaline solution of an amphoteric metal compound (other than zinc) having a hydroxyl ion concentration adapted to produce by anodic action a thin, dense and firmly adherent coating on said zinc base metal. 90

5. The method of producing a coating on a zinc base metal which comprises subjecting the metal as anode to electrolytic treatment in an alkaline electrolyte containing a compound of an amphoteric metal and having a pH of 10 100 to 13.

6. The method of producing a coating on a zinc base metal which comprises subjecting the metal as anode to electrolytic treatment in an alkaline electrolyte containing a compound of an amphoteric metal other than zinc and having a pH of 12 to 13. 105

7. The method of producing a coating on a zinc base metal which comprises subjecting the metal as anode to electrolytic treatment in an 110 alkaline solution of an amphoteric metal hydroxide (or oxide) having a pH of 10 to 13.

8. The method of producing a coating on a zinc base metal which comprises subjecting the metal as anode to electrolytic treatment in an 115 alkaline solution of aluminum hydroxide (or oxide) having a pH of 10 to 13.

9. The method of producing a coating on a zinc base metal which comprises subjecting the metal as anode to electrolytic treatment in an 120 alkaline solution of tin hydroxide (or oxide) having a pH of 10 to 13.

10. The method of producing a coating on a zinc base metal which comprises subjecting the metal as anode to electrolytic treatment in an 125 alkaline electrolyte containing a compound of an amphoteric metal with a hydroxyl ion concentration adapted to produce on said zinc base metal a coherent coating containing a substantial amount of an insoluble compound of the 130 amphoteric metal.

11. The method of producing a coating on a zinc base metal which comprises subjecting the metal as anode to electrolytic treatment in an alkaline solution of an amphoteric metal hydroxide (or oxide) with a hydroxyl ion concentration adapted to produce on said zinc base metal a thin, dense and firmly adherent coating.

12. The method of producing a coating on a zinc base metal which comprises subjecting the metal as anode to electrolytic treatment in an alkaline solution of an amphoteric metal with a hydroxyl ion concentration adapted to yield a dense and adherent coating on the zinc anode while insufficient to completely dominate the anion of the amphotolyte.

13. The method of producing a coating on a zinc base metal which comprises subjecting the metal as anode to electrolytic treatment in an aqueous solution of an alkali zincate with a hy-

droxyl ion concentration adapted to produce on said zinc base metal an adherent coating.

14. The method of producing a coating on a zinc base metal which comprises subjecting the metal as anode to electrolytic treatment in an aqueous solution of an alkali aluminate with a hydroxyl ion concentration adapted to produce by anodic action a firmly adherent coating on said zinc base metal.

10 15. The method of producing a coating on a zinc base metal which comprises subjecting the metal as anode to electrolytic treatment in an aqueous solution of an alkali stannate with a hydroxyl ion concentration adapted to produce by anodic action a firmly adherent coating on said zinc base metal.

20 16. A method of producing a coating on a zinc base metal which comprises subjecting the metal as anode to electrolytic treatment in a solution selected from the group consisting of an alkaline solution of the oxides or hydroxides of zinc, aluminum, beryllium and tin; and an aqueous solution of alkali zincates, aluminates, beryllates and stannates; said solution having a hydroxyl ion concentration adapted to produce by anodic action a thin dense and firmly adherent coating on said zinc base metal.

25 17. A method of producing a coating on a zinc base metal which comprises subjecting the metal as anode to electrolytic treatment in a solution of a compound of a metal that forms an oxide capable of acting as an acid or a base, said solution

having a hydroxyl ion concentration adapted to produce by anodic action a thin dense and firmly adherent coating on said zinc base metal.

18. A method of producing a coating on a zinc base metal which comprises subjecting the metal as anode to electrolytic treatment in a solution of a compound of a metal that forms basic oxides and acid oxides differing in valence, said solution having a hydroxyl ion concentration adapted to produce by anodic action a thin dense and firmly adherent coating on said zinc base metal.

19. A method of producing a coating on a zinc base metal which comprises subjecting the metal as anode to electrolytic treatment in an amphoteric metal electrolyte consisting of an aqueous solution of a salt formed by the combination of a strong base with the hydroxide or oxide of an amphoteric metal, said solution having a hydroxyl ion concentration adapted to produce by anodic action a thin dense and firmly adherent coating on said zinc base metal.

20. A method of producing a coating on a zinc base metal which comprises subjecting the metal as anode to electrolytic treatment in an aqueous solution of a salt selected from the group consisting of aluminates, stannates, chromates, tungstates, and zincates, said solution having a hydroxyl ion concentration adapted to produce by anodic action a thin dense and firmly adherent coating on said zinc base metal.

EDWARD CUSHMAN TRUESDALE.  
ERNEST JOHN WILHELM.

35

110

40

115

45

120

50

125

55

130

60

135

65

140

70

145

75

150